

Jan. 5, 1943.

R. G. QUINN ET AL

2,307,639

METHOD OF MAKING FELTED SHEETS

Filed July 26, 1937

FLOW SHEET



INVENTORS.  
ROBERT G. QUINN,  
HARRY LARISON

BY *Virgil C. Kline*  
ATTORNEY.

## UNITED STATES PATENT OFFICE

2,307,639

## METHOD OF MAKING FELTED SHEETS

Robert G. Quinn, Montclair, and Harry Larison,  
Somerville, N. J., assignors to Johns-Manville  
Corporation, New York, N. Y., a corporation of  
New York

Application July 26, 1937, Serial No. 155,611

3 Claims. (Cl. 92—20)

This invention relates to a felted sheet and the method of making the same. It relates, particularly, to such a sheet impregnated or adapted to be impregnated with asphalt, pitch, or other composition commonly used in the manufacture of prepared roofing.

The product of the invention is useful for such roofing, for flooring felt, or for damping the vibration of automobile bodies or the like.

In the making of felts for these purposes it is customary to use rag fibres mixed with a certain proportion of fibres from old newspapers, commonly referred to as news or news stock. The news fibres are relatively inexpensive as compared to the rag. In addition they require less expenditure for power, to put them into condition suitable for felting. However, only a small proportion of news fibres have been used heretofore in satisfactory felts, because of the tendency of a larger proportion of the news fibres to cause slowness in draining water from the fibres in the felting stage and lack of absorptiveness or porosity of the finished product.

It is an object of the present invention to provide an improved method in which rag fibres are made more free (less slow) at the felting stage. Another object is to provide a method and product in which there may be used a larger proportion of the news stock or other short wood fibres than heretofore, in making a product of satisfactory absorptiveness, strength, tear resistance, and general properties for the purposes mentioned.

Briefly stated, the invention comprises the product resulting from and the method of forming a felt including the rag component thereof in the form of fibres of optimum lengths and, preferably, subjecting the rag fibres to a steaming operation before they are formed into the felted sheet. In another embodiment, the invention includes the steamed rag fibres felted into a sheet and a saturant impregnated thereinto.

The invention will be illustrated by description in connection with the attached drawing which shows a flow sheet of the preferred embodiment of the method for producing the improved product.

The rags selected are of the kind commonly used for making roofing felts, for example, under the designations grades 1, 2, 3, 4, and 5. In the present method there has been used to advantage a mixture of grades 1, 2, 3, and 4, with a heavy preponderance of grades 2, 3, and 4. Because of the process to be described there may be used the relatively cheap grades of rags, containing fibres that in the conventional beating and felt making steps would become too highly hydrated.

The rags selected are subjected to an operation to cut them into little bits, as by being passed through two conventional cutters arranged in series. A typical product from the second of 60

these cutters will be in the form of pieces predominantly one square inch or more in area.

The rags are subjected to a magnetic separation to remove particles of iron or other magnetic material.

The bits of rags are then sent through a spiked-head mill, to produce a tearing and separation, and then through an air cleaner, for separating the rag stock from buttons, buckles, or other heavy objects not previously removed by magnetic separation.

The rags are next passed through a cutter with perforated plates. These plates are in effect screens with holes of selected longest dimension, so that the rag fibres, when reduced to a length to pass through the holes, are removed rather promptly from further action of the cutting mechanism. By proper selection of the size of openings in the screen, there may be passed through 20 the screen fibres of about the length that are desired in the finished felt that is to be made. Thus, there have been used to advantage screens containing closely spaced circular holes varying in different screens between about one-tenth and one-fourth inch in diameter. The cutter includes, suitably, a large rotor with knives mounted lengthwise thereon and an outer casing having a plurality of inwardly extending knives set just to clear the knives on the rotor. The rotor is driven rapidly, say, at a speed of 900 R. P. M., so that there is a draft within the casing which assists in removing the fibres, once they are cut to length to pass through the holes in the screen. Also, the air from the cleaner, which conveys the rags to the cutter, passes through the cutter and promotes the removal of the cut fibres of size to pass the restrictions.

All the equipment that has been described, as well as that to be described later in performing the method and manufacturing the product of the invention, is conventional and is, therefore, not illustrated. For example, the cutter that has been described has been used heretofore in the grinding of certain ores.

The cut fibres, having passed through the perforated plates, are subjected to a treatment to soften the exterior portions thereof without causing hydration throughout the fibres to the extent that is produced by the conventional extended 50 beating operation. Thus, the fibres are subjected to treatment with hot water or steaming. For instance, they may be immersed for a substantial period, for example, from 15 minutes to several hours in water heated within the range extending from approximately 100° C. to the temperature of steam at a pressure of 100 to 200 pounds or so to the square inch. The severity (extent of the effect of steaming) is best within about this range of conditions.

The steamed fibres are mixed with a large pro-

portion of water in a suitable tank, such as a mixing chest. The dilute suspension thus made is passed through a refiner, say a Bauer or Jordan, commonly used in the paper industry, and then over screens which separate the small proportion of oversized material that may be present, due to inefficiencies of the particular machines described.

The suspension, having passed through the screens, is then formed into a felt, as on a Fourdrinier wire or a cylinder mold paper machine, preferably the latter.

In this manner there are eliminated extensive beating and also substantial hydration of the fibres subsequent to steaming.

The water which is separated from the felt on the paper machine, the so-called "white water," is turned to the process, as, for example, through a "white water" storage or chest, to the fibres at some stage in advance of the felting operation.

Wood fibres, if used, are introduced subsequent to the steaming and in advance of the felting operation, as, for instance, into the rag fibres either before they pass through the Jordan or thereafter as shown by the dotted line representing an alternative in the flow sheet. The wood fibres are separately dispersed, as in a pulper or breaker beater, before being mixed with the rag fibres.

Finally, the felt so formed is dried on a usual paper mill drier, after which it may be wound into rolls for future use or it may be used directly.

In case a binder for the fibres is used, the binder is added in fluid form to the stock stream, preferably just before its entry into the refiner. When the binder composition is in the form of an emulsion which must be broken to cause adherence of the binder to the fibres, the chemical employed for this purpose is best added after the binder has been thoroughly mixed with the stock, say, after the mixture comes from the refiner.

A binder that may be used is an aqueous emulsion of asphalt, wax such as paraffin, montan or a mixture thereof, and/or rubber latex. The chemical that is used to break such emulsions and cause separation of the binder on the fibres is usually one that changes the acidity of the composition, suitably by decreasing substantially the pH. Thus, there may be used alum, ferric sulphate, or a small amount of a mineral acid.

The proportions of binder may be varied within limits. There may be used say, 5 to 15% of the binder on the total dry weight of fibres, with just sufficient of the chemical to cause proper breaking, with the establishment of the pH value, for example, at about 5.2.

For most purposes of the present invention the binder is not necessary and is omitted.

With the omission of the binder, there may be used a relatively large proportion of wood fibres in a mixture with rag fibre, in the production of a satisfactory felt for roofing, flooring, or vibration-damping. Thus, there may be used at least 25 to 40 pounds by weight of news fibres to 100 pounds of the felt. The maximum proportion of the news that may be used varies somewhat with the type of the rags selected, the said proportion being larger with the higher grades of rags. The proportion will vary also with the weight of the felt, the proportion that may be used being larger with the lighter felts and smaller with the heavier felts. The term "news" as used herein means repulped waste newspaper, news pulp or the like.

Since 50-pound felts, that is, felts weighing 50 pounds for 480 square feet, are the most impor-

tant in the roofing industry, the properties of such felts will be discussed in detail.

The kerosene value, that is, the measure of the amount of saturant that may be absorbed, is satisfactory as is also the Mullen test. Thus, with 25% of wood fibres on the weight of the felt, the kerosene value and the bursting factor of a typical product are not less than 160 and 50%, respectively, by the standard tests. The kerosene value is obtained by immersing the sheet product in kerosene for one minute, removing the sheet, allowing it to drip for two minutes, weighing the thus drained material and calculating the increase in weight over that of the original sheet as percentage increase in weight. The bursting factor is determined in usual manner by means of a Mullen test and calculations therefrom. The bursting factor represents the bursting strength (pounds per square inch) in the Mullen test divided by the weight of the sheet material being tested (in pounds for 480 square feet) multiplied by 100.

The felt is very free, as determined by testing the fibre stock from which the felt is formed, the fibre stock fed to the machine permitting the rapid flow of water therefrom on the paper machine. In a typical run, the rag fibres, when suspended alone in water and tested by the Motschman test, showed a slowness of practically zero, which means that the freeness is nearly infinite. With a news content of 25% or higher, the mixed fibre stock has been found to have a slowness of not more than 44 seconds for a 2-gram sample used in this test. This freeness is an advantage in the removal of water in the felting stage and, also, in the readiness of impregnation when the felt is later saturated with a material such as asphalt. The Motschman test is made with the standard Motschman tester and involves the following procedure. The two gram sample of fibre stock to be tested is suspended in water in the cylinder of the Motschman tester, the total volume of the suspension being approximately 81 cubic inches and the depth of the suspension in the Motschman cylinder being approximately 10 inches. The bottom of the cylinder is provided with a fine gauze end piece. There is noted the time in seconds required for the water to drain completely through the fibres which become felted on the said gauze, till the outflow becomes discontinuous.

The bulking value of the felt is relatively low for a given kerosene value, which shows that such pores or spaces as are present within the felt are relatively accessible to the saturant. It has been found, for instance, that the felt of bulking factor not in excess of 0.12 will have a kerosene value of at least 160. (The bulking factor is calculated by dividing the thickness of the felt, in hundredths of an inch, by the weight in pounds of 480 square feet.)

As a possible explanation of the combination of desirable properties in the felt, in spite of the high proportion of the inexpensive wood fibres, the screen tests of the rag fibres made as described is of interest.

The rag fibres that have been cut in the cutter with a restricting screen having circular perforations of the preferred diameter of fourteen sixty-fourths of an inch are predominantly within the range of 4-mesh to 28-mesh. Substantially all of the fibres pass through a 4-mesh screen and all but about a fifth or less by weight are retained on a 28-mesh screen. Of the small proportion of material that passes the 28-mesh

screen, most of it is dirt or water-soluble material.

Also, the rag fibres, cut as described, show a half and usually at least two-thirds of their total weight finer than 4-mesh and coarser than 14-mesh, by which is meant the above proportion of the fibres will pass through a 4-mesh and be retained on a 14-mesh screen, in the Johnson classifier used in establishing the screen test data herein.

On the other hand, nearly all the wood fibres used pass through a 14-mesh screen.

Screen tests on the rag fibres as they come from the cutters and on pulped (defibred) news stock that may be used are as follows:

| Screen size, meshes per linear inch | Per cent of total weight of fibres of each kind |       |         |       |
|-------------------------------------|-------------------------------------------------|-------|---------|-------|
|                                     | News                                            |       | Rag     |       |
|                                     | Typical                                         | Range | Typical | Range |
| On 4-mesh screen                    | 0                                               | 0     | 0       | 0-5   |
| Through 4 and on 8                  | 0                                               | 0     | 40      | 10-50 |
| Through 8 and on 14                 | 2                                               | 1-10  | 35      | 30-50 |
| Through 14 and on 100               | 54                                              | 30-60 | 15      | 10-20 |
| Through 100 (partly non-fibrous)    | 44                                              | 35-50 | 10      | 0-20  |

In other words, the rag fibres are comparatively long. For this reason there may be used a large proportion of the relatively fine news fibres, without making the total proportion of all fibres in the very fine grades too large for proper freeness during felting and for adequate strength of the finished felt.

A typical mixture of 35 parts by weight of news and 65 of rag fibres showed the following wet screen analysis at various stages in the manufacturing process:

| Mesh of screen        | Percentage of total weight |                  |          |
|-----------------------|----------------------------|------------------|----------|
|                       | From refiner               | At paper machine | Dry felt |
| Through 4 and on 8    | 10                         | 7                | 8        |
| Through 8 and on 14   | 20                         | 12               | 13       |
| Through 14 and on 100 | 45                         | 51               | 55       |
| Through 100           | 25                         | 30               | 24       |

In the finished felt, the rag fibre component of this typical mixture will show about the following wet screen test:

|                            | Per cent |
|----------------------------|----------|
| On 4 mesh                  | 0        |
| Through 4 and on 8 mesh    | 13       |
| Through 8 and on 14 mesh   | 17       |
| Through 14 and on 28 mesh  | 31       |
| Through 28 and on 100 mesh | 20       |
| Through 100 mesh           | 19       |

Felts so made may be impregnated with the usual saturants, as, for instance, with 100 to 200 parts of asphalt or pitch to 100 parts dry weight of the felt. As such, they make prepared roofing

that is particularly satisfactory in view of its reduced cost.

For best results there may be used, in place of the news stock described, news that has been fractionated by wet screening methods to remove nearly all of the fibres that are so fine as to pass through a 100-mesh screen, as, for example, news showing 80 per cent or more retained on 100-mesh.

The details given are for the purpose of illustration, not restriction, and variations within the spirit of the invention are intended to be included in the scope of the appended claims.

What we claim is:

1. In making a felted sheet, the method which comprises cutting rags to pass through a screen having therein closely spaced holes of largest dimension adapted to pass fibres of the length desired in the finished product and then promptly removing, through the said holes and away from the cutting mechanism, the rag fibres of such length as to pass readily through the holes, subjecting the fibres thus formed to water at an elevated temperature within the range of 100° C. to the temperature of steam at 200 pounds per square inch pressure, with preservation of the said length of the fibres, making a dilute aqueous suspension of the thus treated fibres, forming therefrom a felted sheet, and drying the said sheet.

2. In making a felted sheet, the method which comprises cutting rags to pass through a screen having therein closely spaced holes of longest dimension corresponding approximately to the fibre length desired in the finished product and then promptly removing, through the said holes and away from the cutting mechanism, the rag fibres that are of such length as to pass through the holes, subjecting the fibres thus formed to water at an elevated temperature within the range of 100° C. to the temperature of steam at 200 pounds per square inch pressure with preservation of the said length of the fibres making a mixture, in a large volume of water, of the thus treated fibres with short wood fibres in proportion that is substantial but less than the weight of the rag fibres, forming a felted sheet from the said mixture, and drying the said sheet.

3. In making a felted sheet, the method which comprises cutting rags to lengths suitable for felting on a paper machine, subjecting the cut rag fibres to a steaming operation, suspending the steamed fibres in a large volume of water, forming a felt from the suspension, and then drying the felt, the steaming varying in severity and effect produced between steaming for approximately 15 minutes at about 100° C. and steaming for several hours at temperatures up to those corresponding to steam at a pressure of 200 pounds to the square inch.

ROBERT G. QUINN.  
HARRY LARISON.